

# UNITED STATES PATENT OFFICE.

JOSEPH E. JOHNSON, JR., OF NEW YORK, N. Y.; MARGRAET HILLES JOHNSON EXECUTRIX OF SAID JOSEPH E. JOHNSON, JR., DECEASED.

## PRODUCTION OF FERROCHROMIUM.

1,354,491.

Specification of Letters Patent.

Patented Oct. 5, 1920.

No Drawing.

Application filed July 23, 1918. Serial No. 246,346.

To all whom it may concern:

Be it known that I, JOSEPH E. JOHNSON, Jr., a citizen of the United States, residing at New York city, in the county of New 5 York, State of New York, have invented certain new and useful Improvements in Production of Ferrochromium; and I do hereby declare the following to be a full, clear, and exact description of the invention, 10 such as will enable others skilled in the art to which it appertains to make and use the same.

Ferro-chromium, in so far as I am aware, is now made exclusively in the electric furnace. It was formerly made, to some extent, 15 in the iron blast furnace, but it was found that the limiting percentage of chromium which could be introduced into the alloy obtained in the blast furnace was in the neighborhood of 30%. This is because, at or about that point, an equilibrium is established, in the furnace, limiting correspondingly the reduction of the chromium from its compounds and its introduction into the 20 alloy. The most desirable ferro-chromium alloys for commercial use contain 60% and upward of chromium, and these alloys can not be produced at all in the blast furnace by the processes heretofore employed.

30 My investigations of the iron blast furnace have shown that by supplying a furnace of the same general type as the ordinary iron blast furnace with a blast containing considerably more than the atmospheric percentage 35 of nitrogen, I can so raise the temperature in the hearth as to produce from the usual charge containing the appropriate quantities of carbon, iron, chromium, and silicon (in the usual form of coke, iron ore, chrome ore 40 and silica) as to produce alloys containing 60 or more per cent. of chromium, and that I can simultaneously raise the metallic silicon in the alloy to 10% and upward with the effect of keeping down the percentage of carbon 45 in the alloy, which is essential in the production of the highest grades of ferro-chromium. For the desired result, I do not need a blast consisting wholly of oxygen, but can use a blast containing from 40 to 50 50% of oxygen (and a correspondingly lower per cent. of nitrogen) which is much cheaper to produce than 100% of oxygen.

By varying the amount of increase of oxygen and the amount of decrease of nitrogen 55 in the blast, I am enabled to produce ferro-

chromium containing practically any desired percentage of chromium and to produce it much more cheaply than can be done in the electric furnace. So also, as above noted, the hearth heat may be so far increased as to reduce a considerable percentage of the silica present and cause the silicon thereof to unite with the ferro-chromium with the result of forcing down the carbon content of the alloy. 60

Furthermore, if so desired, the alloy, while still in the liquid condition, but in a separate vessel, may be subjected to the action of oxid of iron or oxid of chromium, or both, with the result that these oxids attack the silicon of the alloy, thereby oxidizing it to silica, which, uniting with a portion of the oxid unreduced, passes off as slag, the metal reduced from the oxid thereupon entering the alloy. By this means I can produce an alloy high in chromium and low in both carbon and silicon. 75

What I claim is:

1. The method of producing in a blast furnace, alloys of iron, high in chromium, 80 which comprises blowing the furnace charge (containing carbon, iron and chromium) with a blast richer in oxygen and poorer in nitrogen than the atmosphere, the relative oxygen and nitrogen content of the blast being so proportioned that an increase in hearth temperature is obtained sufficient to obtain the desired high chromium content in the alloy; substantially as described. 85

2. The method of producing in a blast furnace, alloys of iron, high in chromium and low in silicon and carbon, which comprises blowing the furnace charge (containing carbon, iron, manganese and silicon) with a blast richer in oxygen and poorer in nitrogen than the atmosphere, the relative oxygen and nitrogen content of the blast being so proportioned that an increase in hearth temperature is produced sufficient to obtain the desired high chromium content 95 in the alloy and to likewise increase the content of silicon at the expense of the carbon content of the alloy; substantially as described. 100

3. The method of producing in a blast 105 furnace, alloys of iron, high in chromium and low in silicon and carbon, which comprises blowing the furnace charge (containing carbon, iron, manganese and silicon) with a blast richer in oxygen and poorer in 110

